

# United States Patent Office

2,740,755

Patented Apr. 3, 1956

1

2,740,755

## ELECTROPOLISHING WITH PHOSPHOROUS ACID

Dwight E. Couch, China Lake, Calif., and Abner Brenner, Chevy Chase, Md., assignors to the United States of America, as represented by the Secretary of Commerce

No Drawing. Application April 1, 1953,  
Serial No. 346,294

7 Claims. (Cl. 204—140.5)

(Granted under Title 35, U. S. Code (1952), sec. 266)

The invention described herein may be manufactured and used by or for the Government of the United States for governmental purposes without the payment to us of any royalty thereon in accordance with the provisions of 35 U. S. Code (1952), section 266.

The present invention relates to a method and bath for electropolishing a number of metals, and in particular to electropolishing with a phosphorous acid bath.

It is an object of the present invention to provide a bath for electropolishing a number of different metals.

Another object of the present invention is to provide a bath for electropolishing a number of different metals, which bath can be used at relatively low temperatures.

Another object of the present invention is to provide a method of electropolishing a number of different metals in which phosphorous acid is used as the main constituent of the bath.

In accordance with the present invention the metal to be polished is connected in the electrical circuit as the anode. The cathode of the circuit may be carbon or any other conductive material which is not attacked by the bath. The current densities may range from 5 to 100 amperes/decimeter<sup>2</sup> and the temperature may vary from 20 to 100 degrees centigrade. The particular current density and temperature depends upon the material being polished and the make-up of the bath. The main ingredient of the bath is phosphorous acid, which is available commercially in crystalline 100 percent acid or in 75 percent solution. The crystalline acid melts at 74 degrees centigrade and can be used in the fused state or can be diluted with water or mixed with other acids or organic compounds. A bath which was found to be suitable for polishing copper, brass, nickel, aluminum, cadmium, and stainless steel, was composed of 90 percent by weight of phosphorous acid and 10 percent by weight of water. The acid concentration is not too critical. Electropolishing will take place with concentrations as low as 60 percent.

Solution No. 4 (see Table 2) which contains phosphorous acid, 85-90 percent by weight, water, 0-10 percent, and hydrofluoric acid, 0-5 percent, will polish copper, brass, silver, and molybdenum. This solution will also polish zinc if the hydrofluoric acid concentration is kept at about 2 percent. Higher concentrations of hydrofluoric acid cause a black surface on the zinc.

Although there are many variations possible in the preparation of phosphorous acid electropolishing solutions, the two that seem the most promising are solutions No. 2 and No. 4. Solution No. 4 is made by adding a small amount of hydrofluoric acid to solution No. 2. Solution No. 4, although not usable with all of the metals which solution No. 2 will polish, does polish some metals which solution No. 2 will not polish, and extends the range of metals which can be polished with a bath having phosphorous acid as the basic ingredient.

When aluminum is polished in the 90 percent phosphorous acid bath, solution No. 2, a thick oxide film forms on the surface. This film, which appears as a slight bloom

2

on the surface, can be removed by dipping in dilute sodium hydroxide, leaving a bright surface on the aluminum.

Set out below is a list of metals and the solutions used to electropolish them.

Table 1

| 10 | Metal           | Polish-ing Solution No. | Current Density (amp./dm. <sup>2</sup> ) | Tempera-ture (degrees C.) | Time (min.) |
|----|-----------------|-------------------------|------------------------------------------|---------------------------|-------------|
| 15 | Aluminum        | 2                       | 10-30                                    | 70                        | 2-10        |
|    | Do              | 3                       | 50-100                                   | 20-60                     | 2-5         |
|    | Do              | 5                       | 10-40                                    | room                      | 2-15        |
| 20 | Copper          | 2                       | 10-40                                    | 30-50                     | 2-10        |
|    | Do              | 4                       | 10-40                                    | 30-70                     | 2-10        |
| 25 | Brass           | 2                       | 10-40                                    | 30-90                     | 2-10        |
|    | Do              | 4                       | 10-40                                    | 30-70                     | 2-10        |
|    | Do              | 5                       | 10-40                                    | room                      | 2-15        |
| 30 | Stainless Steel | 2                       | 20                                       | 30-90                     | 10          |
|    | Zinc            | 4                       | 10-40                                    | room                      | 2-15        |
|    | Silver          | 4                       | 10-40                                    | room                      | 2-15        |
| 35 | Molybdenum      | 1                       | 10-40                                    | >80                       | 2-15        |
|    | Do              | 4                       | 10-40                                    | room                      | 2-15        |
|    | Cadmium         | 2                       | 10-40                                    | room                      | 2-15        |
|    | Nickel          | 2                       | 30-40                                    | 30-50                     | 2-15        |

The following solutions were typical baths used for electropolishing.

Table 2

| Solution No.            | H <sub>3</sub> PO <sub>4</sub> | H <sub>2</sub> O | Gly-cerin | 40 per-cent H <sub>2</sub> F <sub>2</sub> | Ethyl Alcohol |
|-------------------------|--------------------------------|------------------|-----------|-------------------------------------------|---------------|
| 1.....percent by weight | 100                            |                  |           |                                           |               |
| 2.....do                | 90                             | 10               |           |                                           |               |
| 3.....do                | 60                             |                  | 40        |                                           |               |
| 4.....do                | 85-90                          | 0-10             |           | 0-5                                       |               |
| 5.....do                | 80                             |                  |           | 10                                        | 10            |

While the invention has been particularly described in connection with several specific bath compositions, it will be understood that various combinations and concentrations of the constituents mentioned, as well as various operating conditions might be employed within the scope of the invention, and that various modifications can be made within the scope of our invention as defined in the appended claims.

We claim:

1. The method of electropolishing various metals selected from the group consisting of aluminum, copper, brass, stainless steel, zinc, silver, molybdenum, cadmium and nickel which comprises connecting the metal to be polished as the anode in a bath consisting essentially of between 60 to 100 percent by weight of phosphorous acid, and passing an electric current of from 5 to 100 amperes/decimeter<sup>2</sup> between said anode and a cathode.
2. The method of electropolishing various metals selected from the group consisting of aluminum, copper, brass, stainless steel, zinc, silver, molybdenum, cadmium and nickel comprising connecting the metal to be polished as the anode in a bath which consists essentially of at least 60 percent by weight of phosphorous acid, and passing an electric current of from 5-100 amperes/decimeter<sup>2</sup> between the anode and a cathode, said bath being maintained at between 20 to 100 degrees centigrade.
3. The method of electropolishing molybdenum which comprises connecting the metal to be polished as the anode in a bath consisting of melted 100 percent phosphorous acid and passing an electric current of between 5 to 100 amperes/decimeter<sup>2</sup> between the anode and a cathode.
4. The method of electropolishing stainless steel which comprises connecting the metal to be polished as the anode in a bath consisting of 90 percent by weight of phosphorous acid and 10 percent by weight of water, and

passing an electric current of between 10 to 40 amperes/decimeter<sup>2</sup> between the anode and a cathode, said bath being maintained at a temperature between 30 and 90 degrees centigrade.

5. The method of electropolishing aluminum which comprises connecting the metal to be polished as the anode in a bath consisting of 60 percent by weight of phosphorous acid and 40 percent by weight of glycerin, and passing an electric current of from 50 to 100 amperes/decimeter<sup>2</sup> between the anode and a cathode, the bath being maintained at temperatures between 20 and 60 degrees centigrade.

6. The method of electropolishing silver, which comprises connecting the metal to be polished as the anode in a bath consisting of 85 to 90 percent by weight of phosphorous acid, 0 to 10 percent by weight of water, and 0 to 5 percent by weight of hydrofluoric acid, and passing an electric current of from 50 to 100 amperes/decimeter<sup>2</sup> between the anode and a cathode, the bath

10 being maintained at a temperature between 30 and 70 degrees centigrade.

7. The method of electropolishing brass which comprises connecting the metal to be polished as the anode in a bath consisting of 80 percent by weight of phosphorous acid, 10 percent by weight of hydrofluoric acid, and 10 percent by weight of alcohol, and passing an electric current of from 10 to 40 amperes/decimeter<sup>2</sup> between the anode and a cathode, the bath being maintained at approximately room temperature.

References Cited in the file of this patent

UNITED STATES PATENTS

15 2,366,712 Faust ----- Jan. 9, 1945

FOREIGN PATENTS

619,336 Great Britain ----- Mar. 8, 1949